

## UNITED STATES PATENT OFFICE

1,959,112

PROCESS OF MANUFACTURING LEATHER  
AND PRODUCTS USED IN CONNECTION  
THEREWITHCharles G. Shaw, Huntsville, and Jacques Hoff-  
man, Toronto, Ontario, CanadaNo Drawing. Application November 15, 1930,  
Serial No. 496,032. Renewed January 17, 1934

9 Claims. (CL. 91—68)

This invention relates to a process of applying coating materials to vegetable tanned leather and more especially to the application of such materials to sole leather subsequently to the compacting of the leather but prior to such finishing operations as "third rolling" and/or brushing.

More particularly, the present invention relates to a further development of the subject matter disclosed in our co-pending application Serial No. 459,103, filed June 3rd, 1930. Prior to our discoveries set forth in the above-mentioned application and in our co-pending application Serial No. 459,104 filed June 3rd, 1930, in connection with the application of coating materials to vegetable tanned leather, such materials when applied to the grain of vegetable tanned leather which had previously been filled with such materials as wax, resin, oil, tanning extract, sugar, and the like, for the purpose of rectifying the unpleasant colour caused by the filling, would lack adhesion and would be removed by subsequent operations in the shoe factory, where it is the practice to soak the leather in water, thus exposing the unpleasant colour beneath.

In our application Serial No. 459,103 referred to above, we have described a process which overcomes this difficulty and provides a finish which satisfactorily adheres to the leather throughout all the subsequent operations to which it is normally submitted either in the process of finishing the manufacture or in being worked in the shoe factory. However, the rather rough treatment to which the coating is subjected in the process of setting out, jacking, rolling, etc. makes it necessary to apply quite a substantial film of material in order that it may withstand the simple wear of the smoothening and finishing operations and at times, if this abrasion is excessive, an additional coating of material has to be applied to bring back the freshness of appearance after the mechanical operations are completed. This may have a tendency to impart to the surface of the finished leather a "painty" appearance and the operations of rolling and pressing after the coating material is applied may result in a darkening of the colour of the leather which is ordinarily corrected in the case of uncoated leather by the use of so-called "sponging compounds" of which there are many on the market, consisting mainly of a slightly alkaline aqueous solution of soaps and sulphonated oil and into which the leather after compaction is quickly dipped and then dried. Subsequently, when the leather is thoroughly dry, it is the usual custom to sub-

mit it to the operation known as "third rolling" which restores the gloss without darkening the colour.

One of the objects of this invention is the application of an adhesive film subsequent to the compacting operations, such film being so thin that while it is sufficient to render the leather uniform in colour it is insufficiently thick to plug the hair holes.

Another object of this invention is the production of sole leather uniform in colour but of extremely rapid and uniform soaking characteristics during the tempering operations in the shoe factory.

In our application Serial No. 459,103 we showed that if the coating materials were applied after the operations of compacting and finishing the leather, adhesion would be unsatisfactory owing to the glazing of the hyaline layer and the plugging of the hair holes. The theory underlying such results is that it is the condition of glaze or unglaze of the surface of the leather or hyaline layer which regulates its absorptive capacity for colloidal matter and thus controls the tendency to adhesion of coating materials applied to it. This explanation is based upon the fact that satisfactory adhesion, so far as we have been able to ascertain has never been obtained by the simple application of the coating materials to leather which has only been rolled, "jacked", "set out" or pressed and many attempts to remove the glossing effects of these operations have been made without rendering the leather in such condition that satisfactory adhesion of the coating materials would result. Simple sponging or washing with water or with the usual sponging compounds was of no avail as, although the appearance of gloss was removed, coating material applied lacked adhesion and was readily removed when the leather was resoaked. Similarly washing the leather with alternate solutions of acids and alkalies gave unsatisfactory results. On the other hand, finished leather when bleached and oiled lightly in a drumming operation would have its surface finish removed and when dried in the usual manner could be coated with materials showing satisfactory adhesion. After such treatment, however, the leather had to be submitted once more to the complete mechanical operations of finishing in order to restore the appearance of finished leather.

We have now found that the objectionable condition of the hyaline layer after the leather has been rolled and pressed can be removed by washing the leather first in a dilute alkali solution and

then in a dilute acid solution such acid solution preferably containing a sulphonated oil of a type which is compatible with the acid solution used. The leather is then dried and the finishing materials applied.

As an example of the manner in which we carry out our invention, the leather is finished and dried and brought to a condition ready for the application of the sponging compound as already 10 described earlier in this specification. It is, however, not treated with the sponging compound but instead is washed on the grain side by applying a solution containing 2% of borax in water at a temperature of about 160° F. to 180° F. 15 This application is conveniently carried out by means of a harness leather blacking machine. The leather is then passed quickly through a solution of a weak organic acid, such as acetic or lactic acid, the strength of the solution being 20 such as to neutralize the effect of the alkali treatment which has darkened the leather, and thus rectify and lighten the colour in much the same manner as is done in the ordinary operation for bleaching the leather. To the acid solution 25 is added about 2% of a sulphonated oil of such a nature that it is not readily thrown out of solution by the acid. "Acidopole" fish oil sulphonated but not neutralized, are examples of the sulphonated oils which we may employ. The 30 leather after being dried is now ready for coating. The materials we prefer are first a priming coat containing pyroxalin and a heavy bodied China wood oil in the proportions of about one part of the former to three parts of the latter made up 35 in the usual lacquer solvents to contain about 12% of solids. This primer is mixed with an equal volume of thinner consisting of the same solvents and is very lightly sprayed on the grain surface of the leather, one gallon of the mixture 40 covering about 300 to 500 sq. feet of surface. After the primer has dried a short time the pigmented coating is applied. This coating composition has the general composition:—

|                   | Per cent |
|-------------------|----------|
| 45 Pigment        | 12.8     |
| Pyroxalin         | 6.0      |
| Dibutyl phthalate | 2.5      |
| Neat's-foot oil   | 7.4      |
| Butyl acetate     | 20.3     |
| Ethyl acetate     | 24.0     |
| 50 Toluol         | 27.0     |
|                   | 100.0    |

the nature of the pigment being varied in accordance with the colour required.

This material is reduced with thinner and a very fine or "mist" coat is applied just sufficient to impart a uniform appearance to the surface of the leather. After the coated material has 60 dried a fine coating of a wax emulsion is sprayed upon the top of the coating composition. This wax emulsion is prepared by melting together two parts of carnauba wax and one part of ceresine wax and slowly stirring in one part of sulphonated castor oil. The mixture is then diluted 65 with water, run through a colloid mill and again diluted with water to the desired spraying consistency. After the wax coating has dried, the leather is "third rolled" and brushed. As the 70 customary brass rolling ball and bed have a tendency to mark the coating, a steel ball or one chromium plated is preferably used and overcomes this difficulty.

We wish it to be understood that we do not confine ourselves to the exact details as outlined in

the above example, as many modifications can be made without departing from the spirit of this invention. For instance, the temperatures of the alkali and acid solutions used can be varied considerably. The alkali solution can be used at 80 room temperature or at any temperature up to that at which it might damage the leather or down to that at which its action upon the leather would be so slow as to demand a prolonged soaking. Similarly the acid solution may be used at 85 any convenient temperature up to that at which the oil will not stay properly in solution or the leather be harmed by the hot water.

Again we may introduce into the alkali solution a small percentage (about 1%) of an ordinary sponging compound into which the leather may be dipped and subsequently treated with an acid solution from which the sulphonated oil has been omitted, subsequently spraying or swabbing on about a 5% solution of sulphonated oil or such emulsifiable mineral oils as are obtained by the addition of triethanolamine soap. We have found that the action of such oil is to prevent the hyaline layer from becoming harsh or "tinny" and aids in securing satisfactory adhesion. 100

We also wish to point out other alkalies may be used in place of the borax referred to. For instance, sodium or potassium hydrates, carbonates or bicarbonates may be used although we prefer borax on account of its less vigorous action 105 on the leather.

Similarly other acids than acetic or lactic may be employed, such as oxalic, sulphurous, sulphuric, and other common organic or inorganic acids but, as some of these harm the leather 110 unless used with caution, we prefer to use acetic or lactic as they are more normal to the tannage of leather.

Further, "third rolling" or "brushing" are not essential to the successful carrying out of our 115 invention although the waxing and "brushing" greatly improve the quality of the finished surface.

We have found that treatment such as that described above is essential if satisfactory adhesion of the coating materials to leather which has already been compacted is to be obtained. It is necessary that the hyaline layer or surface of the leather should be cleansed and held "open" until the coating materials are applied, and we 120 have found that the ordinary sponging compounds applied as such do not accomplish this end. They leave a heavy residue which it has been proven does not function. Borax and the like satisfactorily prepare the hyaline layer but 125 darken and stain the surface, whose colour is only properly restored by the subsequent action of the acid which, however, without the treatment with sulphonated or similar oil assumes a harsh character which it is necessary to overcome 130 if the natural appearance and character of the leather is to be fully restored. This is accomplished by the oil which holds open the structure of the hyaline layer during the evaporation of the water.

Neither does treatment with the acid-oil solution alone function properly. It is necessary that such treatment be combined with the alkali treatment in order to perform the washing treatment quickly enough to prevent the leather from 145 becoming so soaked with water as to require a further compacting operation after the coating composition has been applied. Such an operation would detract appreciably from the advantages to be found from our present invention.

Vegetable tanned leather, such as harness leather or sole leather, finished in accordance with the present invention does not "bruise" or change colour on scuffing or rubbing. It has a very high degree of uniformity of colour and an excellently natural appearance due to the fact that the alkali-acid treatment produces a light and uniform colour which enables a minimum of coating materials to be applied and thus does not detract from the natural appearance of the leather itself.

This minimum of coating materials also means that the leather has excellent soaking properties and in this respect is superior to that produced by either of the processes described in our pending applications. In fact we have produced by this process leather which will soak satisfactorily for working in the shoe factory in from 3 to 10 seconds immersion in water which is of considerable importance in connection with some of the applications of vegetable tanned sole leather.

Having thus described our invention, what we claim is:—

1. A process of manufacturing leather which includes the steps of treating the grain surface of vegetable tanned sole leather or harness leather subsequent to the compacting operation, with a solution of alkali and then of acid containing a sulphonated oil.

2. A process of manufacturing leather which includes the steps of treating the grain surface of the leather as in claim 1, and then applying one or more coatings of waterproof material to the leather in such a manner as not to plug the hair holes.

3. A process of manufacturing leather which includes the steps of treating the grain surface of the leather as in claim 1, and then applying a priming composition containing a pyroxylin and heavy bodied China wood oil dissolved in suitable solvents, and a second coating of a composition containing pyroxylin, neat's-foot oil and a pigment or colouring matter.

4. A process of manufacturing leather which includes the steps of treating the grain surface of the leather as in claim 1, then applying one or more fine coats of waterproof material in such a manner as not to plug the hair holes, and then applying a coating of a wax emulsion and subsequently "third rolling" and/or brushing the leather.

5. A process of manufacturing leather which includes the steps of treating the grain surface of vegetable tanned leather, subsequent to the compacting operation, with a solution of alkali fol-

lowed by treatment with an acid and a sulphonated oil.

6. The herein described process of applying coating materials to vegetable tanned leather following compacting of the leather but prior to such finishing operations as third rolling and/or brushing, said process comprising the following steps (1) washing the leather in a dilute alkaline solution (2) subjecting the washed leather to the action of a solution of a weak organic acid containing a small percentage of a sulphonated oil which is compatible with the particular acid solution used, the strength of said acid solution being sufficient to offset the darkening effect exerted on the leather by the alkaline treatment (3) spraying onto the grain surface of the leather a priming coat containing pyroxylin and a heavy bodied China wood oil dissolved in suitable solvents (4) permitting the priming coat to dry and (5) applying to the previously coated surface a second coating of a composition containing pyroxylin and coloring matter.

7. The herein described process of applying coating materials to vegetable tanned leather following compacting of the leather but prior to such finishing operations as third rolling and/or brushing, said process comprising the following steps (1) subjecting the leather to the action of a dilute alkaline solution containing a small percentage of an ordinary sponging compound (2) treating the leather with a solution of a weak organic acid of sufficient strength to neutralize the darkening effect of the alkaline treatment (3) treating the leather with sulphonated oil to prevent the hyaline layer becoming harsh and to promote adhesion of subsequently applied coating materials (4) then applying to the leather one or more coating compositions containing pyroxylin dissolved in suitable solvents.

8. Vegetable tanned leather, to the grain surface of which has been applied one or more adhesive layers of a composition comprising a cellulose ester and China wood oil and characterized by being uniform in color and capable of being satisfactorily and uniformly soaked in water in 120 from 3 to 10 seconds.

9. Vegetable tanned leather, to the grain surface of which has been applied one or more adhesive layers of compositions comprising a cellulose ester, China wood oil and neat's foot oil and characterized by being uniform in color and capable of being satisfactorily and uniformly soaked in water in 125 from 3 to 10 seconds.

CHARLES G. SHAW.  
JACQUES HOFFMAN. 130

60

135

65

140

70

145

75

150